

## UNITED STATES PATENT OFFICE.

TOMENOSUKE MUTO AND SABURO HIDA, OF KOBE, JAPAN, ASSIGNEES TO KANEKA-FUCHI BOSEKI KABUSHIKI KWAISHA, OF TOKYO-FU, JAPAN.

## PROCESS OF LIQUIDATION OF NATURAL SILK THREADS.

No Drawing. Application filed February 21, 1928, Serial No. 256,059, and in Japan December 15, 1927.

This invention relates to improvements in the process of dissolving natural silk threads and is characterized by the fact that the natural silk is colloidally dissolved in a solution by treating the silk with a solution of magnesium nitrate or other soluble magnesium salts, and then removing the magnesium salts from the solution.

The main object of this invention is to 10 prepare a colloidal adhesive liquid of natural silk from natural raw silk threads, silk yarn, silk waste, old silk cloth or other similar raw silk materials by a simple and economical process, to regenerate silk threads from 15 the liquid or to be utilized in manufacture of plastic materials or painting materials etc.

Heretofore there has been little success in attempts to re-gain silk threads, artificially from liquefied silk, which have high strength 20 and tenacity because threads heretofore formed from solutions of liquefied silk have been brittle.

According to the present invention, these 25 defects are overcome and we are able to obtain threads from a silk solution which possess good strength and tenacity characteristics.

By way of example of carrying out our 30 invention in practice we proceed as follows. About ten parts of magnesium nitrate are dissolved in five parts of water and this solution is heated to a temperature of about 110° C., then two or three parts of waste silk threads divided in several small quantities 35 are successively added, dipped into the said magnesium nitrate solution and stirred gently and dissolved to form a suspending colloidal solution. After that the magnesium salt added is separated and expelled from 40 this suspending solution by dialysis or other ordinary separating method. Dialysis is the preferred method and is accomplished by simply placing the solution in an unglazed earthenware pot surrounded by pure water. 45 Under such conditions, the magnesium nitrate passes through the pot into the water whereas the colloidal silk remains behind. The method of separation by dialysis is a

well known colloidal chemical process and needs no further description. The suspension of natural silk thus formed is now concentrated at a comparatively low temperature. To re-gain silk threads from this concentrated liquid silk the liquid is withdrawn as a fine thread through spinning nozzles in 55 apparatus like that used in artificial silk making industry, and the thus spun threads are then drawn into coagulating solution bath such as acetic acid, methyl-alcohol or other known dehydrating agents. In other cases 60 we may prepare thin paperlike sheets of natural silk by spreading the said concentrated liquid silk over a flat surface such as glass plate and drying the film. A suitable quantity of gelatin, glucose etc. may be added 65 either before or after the expelling of salts to modify the strength and elasticity of the finished thread.

As is shown in the aforesaid explanation 70 one of the characteristics of this invention resides in the use of magnesium nitrate or other soluble magnesium salts as liquefying agents for the natural silk threads. Owing to this reason it is easy to remove the magnesium salts from the colloidal solution of the natural 75 silk and recover a good product having desirable properties and high in stiffness.

While we have shown and described the 80 techniques which we now consider to be the best embodiment of this invention, we desire to have it understood that such changes may be made in the chemical techniques when desired as are within the scope of this invention as claimed, and, accordingly we beg to intend not to be limited as to the details 85 described.

## We claim:—

The method of preparing a colloidal solution of natural silk which comprises dissolving the silk in a solution of magnesium 90 nitrate and then subjecting the solution to dialysis to free it of the magnesium nitrate.

In testimony whereof we have affixed our signatures.

TOMENOSUKE MUTO.  
SABURO HIDA.